

Sept. 13, 1949.

J. G. BROWDER ET AL

2,481,816

METHOD OF FINISHING AROMATIC CONCENTRATES

Filed April 10, 1947



John G. Browder  
Robert M. Love  
Henry G. Schutze  
Richard E. Jannick  
INVENTORS  
BY

J. G. McLean  
ATTORNEY.

## UNITED STATES PATENT OFFICE

2,481,816

## METHOD OF FINISHING AROMATIC CONCENTRATES

John G. Browder, Houston, Robert M. Love, Baytown, Henry G. Schutze, Goose Creek, and Richard E. Tannich, Baytown, Tex., assignors, by mesne assignments, to Standard Oil Development Company, Elizabeth, N. J., a corporation of Delaware

Application April 10, 1947, Serial No. 740,564

2 Claims. (Cl. 196—38)

1

This invention relates to a method of finishing aromatic concentrates containing appreciable quantities (1.0% or over) of olefinic compounds. This invention is particularly adaptable to the finishing of synthetic aromatics produced by the catalytic dehydrogenation of cyclonaphthalenes in which process undesirable by-products such as olefinic compounds are formed which render the concentration and finishing of the aromatic concentrate a difficult operation.

Synthetically produced aromatics resulting from a catalytic dehydrogenation process may be concentrated by distillation and then subjected to liquid sulfur dioxide extraction wherein an extract is produced containing from 70% to 90% aromatics, from 5% to 29% of high boiling paraffinic compounds and from 1% to 5% olefinic compounds. The presence of olefinic compounds in the finished aromatic concentrate renders it unstable because upon storage they tend to polymerize and produce gummy constituents which are not desired if the aromatic concentrate is used as a solvent.

It is known that a toluene-containing fraction produced in a catalytic dehydrogenation process may be treated to remove harmful olefinic bodies by acid-treating the oil, neutralizing the acid-treated oil with a concentrated aqueous solution of caustic alkali, heating the oil to an elevated temperature and hydrolyzing it with an aqueous solution of caustic alkali, and subsequently distilling the treated oil under controlled conditions to produce a stable nitration grade toluene concentrate. This process is disclosed and claimed in U. S. Patent 2,400,373.

Although the above-mentioned process has been found to be particularly suitable for finishing nitration grade toluene concentrates, it is not applicable for finishing all types of aromatic concentrates. For example, the higher boiling aromatics such as the xylenes may be treated by the above-mentioned process to produce a concentrate which is not entirely satisfactory from the standpoint of stability. It is also sometimes desired to produce an even more stable toluene concentrate than is produced by the above-described procedure.

It is the main object of the present invention to provide a method for treating an aromatic-containing oil.

It is a further object of this invention to treat aromatic-containing oils by a procedure permitting the production of an aromatic concentrate having improved stability characteristics.

Briefly, our invention comprises acid treating

2

an aromatic-containing fraction under controlled conditions to remove substantial portions of olefinic compounds, separating acid sludge from the treated material, neutralizing easily neutralized constituents in the acid treated material in the presence of an alkaline solution, hydrolyzing the alkaline washed material at elevated temperatures and carefully controlled contact times with an alkaline solution of carefully adjusted concentration, separating the hydrolyzed material, adding to it an alkaline material and distilling it under carefully controlled conditions such that acidic materials released during the distillation are neutralized and recovering an aromatic concentrate from the distillation operation which is inhibited with a phenolic material to obtain an aromatic concentrate of improved stability characteristics.

We have found that an aromatic-containing fraction of the character above-described may be treated to improve its stability to a desired degree by a process including the following steps. The temperature of the extract from the sulfur dioxide extraction process is adjusted to approximately 80° F. and the extract is then acid treated in a two-stage acid treater. Fresh sulfuric acid is employed in the second stage and acid sludge withdrawn from the second stage is utilized to pretreat the extract in the first stage. Following the acid treatment, caustic soda solution of from 18° to 20° Bé. is employed to neutralize the acid oil. The neutralized acid oil is then hydrolyzed at a temperature in the range of 300° to 325° F. in the presence of 18° to 24° Bé. caustic soda solution and then separated from the caustic soda solution by settling. The hydrocarbon material withdrawn from the settling stage is admixed with saponified petroleum phenols or sodium naphthenates and distilled to remove an aromatic concentrate as a condensate fraction. The condensate fraction is then inhibited by the addition of petroleum phenols or other inhibitor and a finished aromatic concentrate of improved stability is thus obtained. The operation of the hydrolyzing step in the above finishing procedure is of prime importance. Two different types of sulfonated material are contained in the finished extract charged to this unit. These are the alkyl sulfates which are easily hydrolyzed in the presence of steam or hot caustic and the aromatic sulfonates and chemically neutral sulfonated compounds which are extremely difficult to hydrolyze by steam or hot caustic. It is necessary to remove both types of sulfonated compounds or to neutralize them in

the distillation step in order to prevent the liberation of free sulfur dioxide in the distillation step which will be contained in the finished aromatic concentrate and which will render this contaminated concentrate unstable in storage with respect to acid wash color and sometimes original color.

In order to explain the present invention more fully, the preferred treating procedure will be described in conjunction with the drawing in which the single sheet is in the form of a diagrammatic flow sheet.

Referring now to the drawing, an aromatic-containing mixture such as is obtained from a sulfur dioxide extraction plant is passed through line 11 to incorporator 12, acid sludge being introduced into the liquid stream flowing through line 11 by means of line 13. An admixture of acid sludge and the aromatic-containing stock is withdrawn from incorporator 12 by line 14 and passed into settling vessel 15. An acid sludge layer is withdrawn from vessel 15 by line 16 and a hydrocarbon fraction is withdrawn by line 17, admixed with fresh acid from line 18 and passed into incorporator 19 where thorough admixture of the fresh acid with the hydrocarbon fraction results. From incorporator 19, the mixture passes through line 20 to a second settling vessel 21. Acid sludge from the lower portion of vessel 21 is recycled through line 13 containing pump 22 and the hydrocarbon fraction is withdrawn by line 23, has an alkali metal hydroxide solution such as caustic solution added thereto by line 24 and passes into incorporator 25. A mixture of caustic and hydrocarbons is withdrawn from the incorporator 25 by line 26 and passes into settling vessel 27. Caustic from the lower portion of vessel 27 is withdrawn through line 24 and is recycled by means of pump 28. If desired, spent caustic may be withdrawn from the recirculating line by outlet 29 and fresh caustic may be added to the recirculating line by inlet 30.

The hydrocarbon fraction from vessel 27 may be withdrawn through line 31 to intermediate storage vessel 32. Hydrocarbon from vessel 32 is withdrawn through line 33, sent through pre-heater 34 where it is heated to a temperature in the range of 300° to 325° F. and then passed by pipe 35 to vessel 36. Vessel 36 is arranged to allow intimate contacting of immiscible fractions therein and the settling of said fractions and to this end is provided with recirculating line 37 containing pump 38, and heater 38'; line 37 discharges into vessel 36 through spray nozzles 39. Recirculating line 37 is provided with outlet 40 and inlet 41 for the rejection of spent caustic and the addition of fresh caustic, respectively.

The aromatic-containing fraction injected into vessel 36 by means of line 35 is thoroughly admixed with an alkali metal hydroxide solution such as caustic soda solution having a gravity in the range of 18° to 24° Bé. and at a temperature in the range of 300° to 325° F. for no less than ten minutes. This admixing step is carried out in the apparatus disclosed by contacting the aromatic-containing fraction injected into vessel 36 with 18° to 24° Bé. caustic which is dispersed through spray nozzles 39 at a high velocity. Heater 38' may be used to maintain the temperature of the mixture in the drum at the desired operating temperature of 300° to 325° F. The retention time of the aromatic-containing fraction in the mixing section of the drum must be a minimum of ten minutes. After the mixing period the hydrocarbon caustic mixture is con-

ducted to the settling section of the drum wherein the two phases are allowed to separate. The aromatic-containing fraction is withdrawn from the vessel continuously by means of line 42.

To obtain an aromatic fraction of satisfactory stability, the charge within vessel 36 must be maintained in intimate admixture with the caustic soda for a minimum period of ten minutes and the total time of contacting and settling must not be less than 1 hour at 300° F. or one-half hour at 325° F. It is preferable to renew the caustic soda solution in vessel 36 when its total sulfate content has increased to 40,000 parts per million although, if desired, the sulfate content may be allowed to increase to 60,000 parts per million before the renewal step. In ordinary operations the caustic must be renewed when from 300 to 500 barrels of aromatic extract have been treated per barrel of caustic.

The aromatic-containing fraction passing through line 42 has added to it a portion of saponified petroleum phenols, sodium naphthalenes, or other basic material from line 47, pump 48, and line 49. The quantity of saponified petroleum phenols or other material added through line 49 will vary depending on the tendency of the material undergoing distillation to release sulfur dioxide. As a rule, it is desired to add from 30 to 50 gallons of such material per 1,000 barrels of concentrate. The concentrate containing the saponified material then passes into distillation zone 43 where it is separated by distillation. A light overhead fraction may be removed from the zone through line 44, a side stream consisting of the desired aromatic concentrate is removed via outlet 45 and a bottoms fraction is removed through line 46. To prevent excessive decomposition of sulfonated compounds in the distillation column, it is desirable to heat the hydrocarbon fraction no higher than about 525° F. in the distillation zone. This is true even though an alkaline material is present in the hydrocarbons undergoing distillation.

It is to be understood that zone 43 may comprise one or more precise fractionation towers. For example, this zone may comprise two efficient distillation towers with the finished aromatic concentrate being recovered as an overhead fraction from the second of the two towers. Inhibitor, such as petroleum phenols, is withdrawn from tank 50 through valve 51 and line 52 to combine with the aromatic concentrate passing through line 45. The finished stabilized aromatic concentrate may be withdrawn through line 53 to a suitable storage means not shown. Usually approximately two to fifteen pounds of inhibitor per 1000 barrels of the finished aromatic concentrate is sufficient to insure the production of a stable product.

The amount of sulfuric acid employed in the acid treating step will depend on the molecular weight of the aromatics being treated and on the amount of olefinic materials contained in the concentrate. It is known that the low molecular weight aromatics such as benzene or toluene do not sulfonate as easily as do the high molecular weight aromatics such as xylenes because the latter types contain a greater number of alkyl groups which cause the aromatic rings to be more reactive to the sulfuric acid. The acid consumption during the acid treating process is, therefore, somewhat lower for the low molecular weight aromatics than it is for the high molecular weight aromatics. The amount of sulfuric acid used can be designated by the term "pounds of acid per

bromine number barrel." In other words, if a stock has a 5 bromine number and is acid treated with 25 pounds of acid per barrel of stock, the acid treat is 5 pounds of acid per bromine number barrel. A typical benzene concentrate usually requires as little as one to two pounds of acid per bromine number barrel and a toluene concentrate, from 2.5 to 3 pounds of acid per bromine number barrel.  $C_8$  and  $C_9$  aromatics usually require approximately 4 to 5 pounds of acid per bromine number barrel and the higher boiling aromatics will require more acid per bromine number barrel depending on their molecular weight and the ease with which they sulfonate.

As previously mentioned, the alkaline material added to the concentrate in line 42 may suitably be a partially or completely saponified petroleum phenols fraction such as sodium phenolates or may comprise alkali metal salts of naphthenic acids derived from petroleum fractions. The chief function of this material is to neutralize sulfur dioxide formed during the distillation step from acidic materials not removed during the hydrolysis operation. The inhibitor added to the distilled aromatic concentrate may suitably be petroleum phenols, an amino phenol, such as *N*-butyl-*p*-aminophenol, or a phenylenediamine, such as *N,N'*-di-*sec*-butyl-*p*-phenylenediamine or their mixtures.

A typical example of a treatment of an aromatic-containing fraction comprising predominately  $C_8$  and  $C_9$ , aromatics resulting from catalytic dehydrogenation will now be given. A fraction having a boiling range of 250° to 500° F. and consisting of 75.4% aromatics, 20% paraffinic compounds, and 4.6% olefinic compounds with a bromine number of 5.8 was treated with 25 pounds per barrel of 96% sulfuric acid. The acid-treated oil was then contacted with 20° Bé. caustic soda solution in an amount equivalent to about 4.3 pounds of sodium hydroxide per barrel of oil. The aromatic-containing charge was then heated to a temperature of about 315° F., admixed with 1.5 volumes of 20° Bé. sodium hydroxide solution at a temperature of 325° F. and kept in intimate contact therewith for ten minutes in the mixing zone of the hydrolyzer drum. The caustic was separated from the mixture in the settling drum of the hydrolyzer and the aromatic-containing fraction was withdrawn from the hot caustic solution after a total contact and settling time of about one-half hour at 325° F.

A portion of the aromatic concentrate was then distilled to separate a fraction containing 99% aromatics and having a bromine number of 0.1. The distilled aromatic concentrate was then tested for acid wash color. An accelerated oxidation test was then made in which the hydrocarbons were heated for various periods of time in the presence of an oxygen-containing gas under carefully controlled conditions, and the acid wash color was again tested. The results of these tests are shown as follows:

|                                   | Acid wash color |
|-----------------------------------|-----------------|
| Original                          | 1-2             |
| Accelerated oxidation test—after— |                 |
| 4 hours                           | 6-7             |
| 8 hours                           | 8-9             |
| 12 hours                          | 9-10            |
| 16 hours                          | 9-10            |
| 20 hours                          | 12-13           |
| 24 hours                          | 14              |

A sample of the distilled aromatics was also placed in storage for a period of 19 days after

which time the acid wash color was found to have increased from 1-2 to 11.

The acid wash color of the aromatic concentrate was determined by agitating 21 cc. of the concentrate with 7 cc. of water white 96% sulfuric acid for 20 seconds in a 30 cc. square bottle. The mixture was then settled for 15 minutes and the color of the acid layer compared with the color of a series of standard solutions. An acid wash color of 6-7 indicates that the color of the acid layer is intermediate the color of standards 6 and 7. The higher the color, the poorer the stability of the oil being treated.

The accelerated oxidation test is carried out by placing 500 cc. of oil in a one liter, round-bottom flask and placing the flask in a bath maintained at a temperature of about 200° F. Air is bubbled through the oil in the flask at a carefully controlled rate for 24 hours. Every 4 hours during the oxidation period a sample of the oil is removed and tested for acid wash color.

It is seen that the aromatic concentrate finished by the above procedure was very unstable since the acid wash color should not be above about 4 after 24 hours' accelerated oxidation.

Another portion of the sample of distilled concentrate was inhibited with petroleum phenols and the acid wash color of the inhibited product was tested after being subjected to an accelerated oxidation test for various periods of time. The results of these tests are shown as follows:

|                                   | Petroleum phenols, lb./1000 bbl. | 2   | 10 |
|-----------------------------------|----------------------------------|-----|----|
|                                   | Acid wash color                  |     |    |
| Original                          | 1-2                              | 1-2 |    |
| Accelerated oxidation test after— |                                  |     |    |
| 4 hours                           | 2                                | 2   |    |
| 8 hours                           | 3-4                              | 2   |    |
| 12 hours                          | 5                                | 2   |    |
| 16 hours                          | 5                                | 2   |    |
| 20 hours                          | 5-6                              | 4   |    |
| 24 hours                          | 6                                | 4-5 |    |

It is seen that the addition of from 2 to 10 pounds of inhibitor per 1000 barrels of the aromatic concentrate greatly improved the stability of this material.

A portion of the hydrocarbons subjected to the above caustic hydrolysis procedure was then distilled in the presence of 39 gallons of saponified petroleum phenols per 1,000 barrels of feed and the resulting aromatic concentrate removed from the distillation tower was inhibited with 10 pounds of petroleum phenols per 1000 barrels. The inhibited concentrate was then subjected to an accelerated oxidation test and the acid wash color of the concentrate was determined after various oxidation times. These tests are shown as follows:

|                                   | Acid wash color |
|-----------------------------------|-----------------|
| Original                          | 2-3             |
| Accelerated oxidation test after— |                 |
| 4 hours                           | 3-4             |
| 8 hours                           | 2-3             |
| 12 hours                          | 2-3             |
| 16 hours                          | 2-3             |
| 20 hours                          | 3-4             |
| 24 hours                          | 3-4             |

It is seen that the distillation of the concentrate in the presence of saponified petroleum phenols combined with the inhibiting operation produced a finished concentrate which is more stable than that produced by distilling without the addition of petroleum phenols followed by inhibiting the material.

7 It is mentioned that increasing the acid treat in the above example to 40 pounds of acid per barrel produced a concentrate which after caustic treating, hydrolysis, and distilling was not improved in acid wash color as compared to that treated with 25 pounds of acid per barrel. It is indicated, therefore, that the critical phase of the treating procedure is that of preventing sulfur dioxide from carrying over into the finished aromatic concentrate in appreciable quantities and of inhibiting the finished aromatic concentrate to prevent any small quantities of acidic materials therein from deleteriously effecting the stability of the finished product.

Having fully described the present invention, what we wish to claim is:

1. A process for the treatment of a hydrocarbon oil comprising a major portion of aromatics and a minor portion of olefins including the steps of admixing said oil with concentrated sulfuric acid at approximately atmospheric temperature to form an acid sludge and separating the acid sludge therefrom, subsequently admixing said oil with caustic soda solution of 18° to 200 Bé. at approximately atmospheric temperature and separating said oil from said caustic soda solution, heating the oil to a temperature in the range of 300° to 325° F., intimately contacting said oil with caustic soda solution of 18° to 24° Bé. for less than ten minutes and subsequently separating the hot caustic soda solution from the oil with a total contacting and separating time of not less than one hour at 300° F., adding to said separated oil an alkali metal salt of petroleum naphthenic acids, distilling said mixture at a temperature no higher than 525° F., removing an aromatic concentrate as a side stream from said distillation, and inhibiting said aromatic concentrate.

2. A process for the treatment of a hydrocarbon oil comprising a major portion C<sub>8</sub> and C<sub>9</sub> aromatics and a minor portion of olefins including the steps of admixing said oil with concentrated sulfuric acid at approximately atmospheric tem-

8 perature to form an acid sludge and separating the acid sludge therefrom, subsequently admixing said oil with caustic soda solution of 18° to 20° Bé. at approximately atmospheric temperature and separating said oil from said caustic soda solution, heating the oil to a temperature in the range of 300° to 325° F., intimately contacting said oil with caustic soda solution of 18° to 24° Bé. for no less than ten minutes and subsequently 10 separating the hot caustic soda solution from the oil with a total contacting and separating time of not less than one-half hour at 325° F., admixing said separated oil with from 30 to 50 gallons of an alkali metal salt of petroleum naphthenic acids per 1000 barrels of oil, distilling said oil at a temperature no higher than 525° F., removing a low boiling fraction as overhead and a desired aromatic-containing fraction as a side stream, and adding to said aromatic-containing fraction from 15 20 to 15 pounds of a phenolic inhibitor per 1000 barrels of said fraction.

JOHN G. BROWDER.  
ROBERT M. LOVE.  
HENRY G. SCHUTZE.  
RICHARD E. TANNICH.

#### REFERENCES CITED

The following references are of record in the file of this patent:

#### UNITED STATES PATENTS

| Number        | Name         | Date           |
|---------------|--------------|----------------|
| 1,761,328     | Chappell     | June 3, 1930   |
| 2,006,407     | Pew          | July 2, 1935   |
| 3,5 2,033,297 | Pott         | Mar. 10, 1936  |
| 2,400,373     | Schutze      | May 14, 1946   |
| 2,408,011     | Walsh et al. | Sept. 24, 1946 |

#### FOREIGN PATENTS

| Number  | Country       | Date         |
|---------|---------------|--------------|
| 414,644 | Great Britain | Aug. 7, 1934 |

**Certificate of Correction**

September 13, 1949

Patent No. 2,481,816

JOHN G. BROWDER ET AL.

It is hereby certified that error appears in the printed specification of the above numbered patent requiring correction as follows:

Column 7, line 24, for "18° to 200 Bé." read  $18^{\circ}$  to  $20^{\circ}$  Bé.;  
and that the said Letters Patent should be read with this correction therein that the same may conform to the record of the case in the Patent Office.

Signed and sealed this 31st day of January, A. D. 1950.

**[SEAL]**

**THOMAS F. MURPHY,**  
*Assistant Commissioner of Patents.*